

## UNITED STATES PATENT OFFICE

2,298,917

## MODIFICATION OF FATTY OILS

László Auer, East Orange, N. J.

No Drawing. Application February 5, 1942,  
Serial No. 429,661

15 Claims. (Cl. 260—407)

## GENERAL FIELD OF INVENTION

This invention relates to the modification of organic isocolloids. More particularly, the invention is concerned with the bodying of fatty oils.

The subject matter claimed herein is divided from my copending application Serial No. 318,650 of which the present application is a continuation-in-part, and said subject matter is disclosed not only in said application 318,650 but also at least in part in certain other prior applications, especially Serial No. 359,425 (now Patent No. 2,213,944), and Serial No. 143,786 (now Patent No. 2,189,772).

Organic isocolloids are colloidal substances in which the dispersed phase and the dispersion medium are both of the same chemical composition, although present in a different physical state. In the bodying of fatty oils (which are organic isocolloids) the relation between the dispersed phase and the dispersion medium is altered, the dispersed phase being increased and the dispersion medium correspondingly decreased.

In accordance with various of my prior applications, including those mentioned above, various different methods are disclosed for modifying organic isocolloids, and especially for bodying fatty oils. In general, the modification is brought about by heating the isocolloid in the presence of a modifying agent.

In the prior applications, various different generic and sub-generic classes and specific modifying agents are disclosed; and, in addition, there are also disclosed variations in process. Different modifying agents or groups thereof, and also variations in process, effect different results, some being of importance for certain purposes and some for other purposes.

The present application is particularly concerned with the modification of fatty oils by means of polar compounds, i. e., modifying agents containing a positive charge in one part of the molecule and a negative charge in another part of the molecule, or capable of orienting their different radicals in opposite directions on an interface of liquid-gas, liquid-solid, or liquid-liquid. More specifically, the invention is concerned with that class of modifying agents which I have termed "2-radical" type, i. e., having within the molecule an acidic inorganic residue and an organic residue. By an acidic inorganic residue I mean a residue capable of yielding an inorganic acid upon the addition of one or more hydrogen atoms or OH groups.

The subject matter claimed herein relates to the use of 2-radical type modifying agents in which the acidic inorganic residue contains sulphur and is capable of yielding an inorganic sulphur-containing acid upon the addition of hydrogen or OH groups, for instance from a water

molecule, this particular sub-group of agents having certain distinctive characteristics distinguishing it from other modifying agents in the general class, in which the inorganic radical does not contain sulphur. The distinctive characteristics will be pointed out more fully hereinafter.

## THE STARTING MATERIAL

The fatty oils and similar materials with which the present application is especially concerned find one of their most important uses in the coating materials and plastics industries, especially the paint and varnish industry, where oils having good body and drying power are very important. The improved products produced in accordance with this invention also have many other uses.

A list of typical oils which may be advantageously modified by my invention is as follows:

|    |                       |               |
|----|-----------------------|---------------|
| 20 | Tung oil              | Rapeseed oil  |
|    | Castor oil            | Walnut oil    |
|    | Linseed oil           | Pine seed oil |
|    | Fish oil (train oils) | Corn oil      |
|    | Poppyseed oil         | Olive oil     |
| 25 | Sunflower oil         |               |

15 The ease of bodying or modification, under equal conditions, decreases in the order given. That is, the first mentioned oils are most extensively bodied or modified by my methods, while the oils 30 at the end of the series are modified to a lesser body. However, it should be also mentioned that by the employment of suitable modifying agents in my methods, even the last mentioned oils (those at the end of this series) can be profoundly modified or bodied, as well as those oils appearing in the first of the series.

The foregoing listed, and other fatty oils may be classified as follows:

| 40 | Drying oils.     | Semi-drying oils               |
|----|------------------|--------------------------------|
|    | Tung oil         | Sunflower oil                  |
|    | Oiticica oil     | Poppyseed oil                  |
|    | Linseed oil      | Soya bean oil                  |
| 45 | Perilla oil      | Walnut oil                     |
|    |                  | Rapeseed oil                   |
|    |                  | Pine seed oil                  |
| 50 | Non-drying oils. | Special oils                   |
|    | Olive oil        | Hydroxylated; castor oil, etc. |
|    | Corn oil         | Fish oils (train oils)         |
|    | Cottonseed oil   |                                |
|    | Coconut oil      |                                |

55 The fish oils are mixtures of non-drying and drying triglycerides. In accordance with the invention, the oils referred to may be treated per se, or they may be treated in mixtures containing more than one 60 such oil, or containing other materials. For in-

stance, synthetic resins containing natural resins or acids of fatty oils and of resins, may be modified in accordance with the invention.

In addition, separated fractions of fatty oils (for instance, the better drying fractions) may be used as starting materials, either alone or mixed with other oils.

The process of the present invention may, in fact, be used in connection with fatty oils themselves, fatty acids, esters of fatty acids, and various materials containing the same, and it is to be understood in connection with the appended claims that where reference is made to treating fatty oils, the language is not to be understood as limited to treatment of fatty oils per se, since essentially the same reaction takes place in the case of treatment of the fatty acids, esters thereof, etc.

#### THE MODIFYING AGENT

As hereinbefore mentioned, the present application is particularly concerned with the use of modifying agents having within the molecule an acidic inorganic sulphur-containing residue, and an organic residue, the inorganic residue being capable, upon the addition of one or more hydrogen atoms or OH groups, of yielding a sulphur-containing acid.

With reference to the yielding of a sulphur-containing acid, it may be mentioned that although I believe that that reaction takes place during the treatment of the oil, in some cases and conditions the reaction may not occur to any considerable extent. Nevertheless, the treating agents herein contemplated as suitable, are those which have the potential capability of yielding the corresponding sulphur-containing acid, upon the addition of hydrogen to the inorganic residue.

In fuller explanation of the capability of yielding the sulphur-containing acid, it is to be understood that the acid may be produced in different ways with different compounds. Thus, in some instances, (a) the addition of OH groups is required, these normally being derived from H<sub>2</sub>O, the remaining H atom combining with the organic part of the molecule; with other compounds, (b) the addition of hydrogen is sufficient; with still other compounds, (c) the addition of hydrogen (H<sub>2</sub>) is required, being derived from H<sub>2</sub>O, the remaining oxygen atom combining with the organic part of the molecule; and finally, the compound may be of such nature that (d) mere splitting-up thereof, as by the application of heat, may yield the sulphur-containing acid. An example of each one of these four types, selected from groups given hereinafter, is as follows:

- (a) Beta-naphthol 3:6:8 sulphonic acid.
- (b) Diamino-diphenyl sulphide.
- (c) Thiocarbanilide.
- (d) Diphenylamine sulphate.

From the above it will be noted that although in some instances, heat alone may suffice to yield the sulphur-containing acid, in most instances the addition at least of hydrogen is required, although the hydrogen may be derived in different ways with different compounds. In any event, all of the materials in question have in common the capability of yielding the sulphur-containing acid under the normally prevailing reaction conditions.

Agents in this class facilitate the heat bodying of fatty oils. More particularly, these agents are outstanding in increasing the rate of bodying. 75

At the same time, this class of modifying agents is of advantage since it promotes liberation of water from the reaction mixture.

Modifying agents coming within this general group may be classified in various ways, the organic sulphonic acids and the sulphonyl chlorides representing two important (though not all) sub-groups.

Sulphonic acids and their derivatives increase alkali resistance of oils per se, or in varnishes.

Sulphonic acids with amino- and/or hydroxy-substituents are especially advantageous, since products of lighter color may more readily be secured therewith, than with other sulphonic acids.

Examples of the sulphonic acids and sulphonyl chlorides are as follows:

- Benzene sulphonic acid,
- p-Toluene sulphonic acid,
- 2:5 dichlorobenzene sulphonic acid,
- m-Xyldine sulphonic acid,
- p-Toluidine-m-sulphonic acid,
- Naphthalene 2:6 disulphonic acid,
- Beta-naphthol 1:5 disulphonic acid,
- 25 Beta-naphthol 3:6:8 trisulphonic acid,
- Beta-naphthylamine 3:6:8 trisulphonic acid,
- 2:1 naphthylamine sulphonic acid,
- 2:6 naphthylamine sulphonic acid,
- 1:4 naphthylamine sulphonic acid (naphthionic acid),
- 30 Benzene sulphonyl chloride,
- p-Toluene sulphonyl chloride,
- Naphthalene-1-sulphonyl chloride,
- 2-phenylamino-8-naphthol-6-sulphonic acid,
- 35 Alpha-naphthyl sulphamic acid,
- Sulpho salicylic acid.

Inorganic salts of organic bases may also be used, for instance—

- 40 Diphenylamine sulphate,
- Diaminodiphenylamine sulphate,
- Aniline sulphate,
- Amino-azo-benzene sulphate.

45 Still further, esters of inorganic acids (containing sulphur and capable of yielding a sulphur-containing acid) may be employed, such as—

- 45 Methyl-p-toluene sulphonate,
- Ethyl chlorosulphonate,
- 50 Dimethyl sulphate.

Some thio- compounds may be used, for instance—

- 55 Thiocarbanilide,
- Diamino-diphenyl sulphide.

From the foregoing it will be seen that certain treating agents in the class herein claimed may be relatively complex compounds incorporating, in addition to the sulphur-containing residue, other residues such, for instance, as a halogen-containing residue capable of yielding a halogen-containing acid upon addition of hydrogen, or a nitrogen-containing residue capable of yielding a nitrogen-containing acid upon addition of hydrogen or OH groups. In such cases, the treating agent partakes somewhat of the characteristics of the halogen or nitrogen, as well as of the sulphur-containing acid.

70 In this connection it is pointed out that in copending applications filed concurrently herewith (Serial Nos. 429,662 and 429,663), I have disclosed and claimed other 2-radical type treating agents having within the molecule a halogen-containing residue or a nitrogen-containing residue. In certain instances, therefore, some of

the treating agents herein referred to also belong to a group of agents claimed in a copending application, although in this event such a compound treating agent manifests not only the distinctive characteristic of the group claimed herein, but also the distinctive characteristic of the group claimed in said copending application.

#### TREATMENT CONDITIONS

In carrying out the process, the treating agent and the oil are first mixed together in any suitable way. Treating agents of different physical characteristics, such as consistency, naturally require different technique for mixing. These matters need not be considered in detail herein since they are fully disclosed in my copending application Serial No. 318,650.

The mixing may be effected in the cold, i. e., at room temperature; or may be effected at elevated temperatures, for instance at some temperature in the preferred range of reaction temperature.

While the quantity of treating agent may range anywhere from a minor amount (for instance, a fractional percentage) up to about 30%, ordinarily the amount required is relatively small, not usually more than about 10%. In general, the degree of modification of the oil increases with increase in the amount of modifying agent used. The lower limit depends somewhat on the particular agent and also on the particular oil being treated, although at least some modification is observable from even minor fractional percentages, going down as low as .01%.

The treatment temperature may also be varied over a considerable range, depending upon the nature of the treating agent and of the oil, as well as on the character and extent of modification desired. In general, the temperature should be considerably above room temperature, but not above the boiling or decomposition point of the oil. A good working range is from about 100° to about 350° C., and preferably above about 200° C.

The time of treatment is also a variable, depending upon the treating agent, the starting material and the result desired. In general, increasing the time of treatment results in more extensive modification, and in most instances the treatment at reaction temperature should be continued for at least 30 minutes, and preferably for several hours.

The reaction may take place either in an open or in a closed vessel; and either at sub-atmospheric, at atmospheric, or at super-atmospheric pressure. Different results are secured under various of these conditions, as is brought out more fully in my copending application Serial No. 318,650.

With reference to the foregoing statement of treatment conditions, it is pointed out that these matters are discussed only briefly herein, since they are fully disclosed in my copending application Serial No. 318,650, to which reference may be had for further information. This is also true as to the supplemental matters discussed just below.

#### SUPPLEMENTAL TREATMENT CONDITIONS AND AGENTS

My processes may be practiced in the absence of any additional material, other than the polar compound. However, I have found it is advantageous in some cases to incorporate the polar compound in the presence of additional materials which facilitate its incorporation and the modification of the organic isocolloid. For in-

stance, the polar compound may be incorporated in the presence of various organic bodies such as the purely organic additions mentioned post or organic solvents. Again metal soaps may also be added; for instance siccatives (driers) such as the resinites and linoleates of metal compounds and metal oxides, commonly used in the varnish industry, as is mentioned in Serial No. 143,786. Further, sulphur or sulphur compounds, such as sulphur chloride, etc., may also be used in these processes and added in addition to the polar compound during the reaction or as an after treatment. The sulphur or sulphur compounds effect further modification and produce sulphurized products. The temperature usually employed for modification (above 200° C.) being substantially above normal vulcanization temperatures, the effect of the sulphur treatment at modifying temperatures is quite different from vulcanization.

However, I may also effect vulcanization of my modified products in an after treatment, so as to produce solid, coherent and elastic products, similar in some characteristics to ordinary rubber. Sulphur may be used for this purpose and may be added as such, or in the form of a sulphur compound, such as sulphur chloride, etc. The action of the sulphur is analogous to that which takes place in the vulcanization of rubber. Thus, accelerators or activators (zinc oxide, etc.) or both, such as usually employed in the vulcanization of rubber, may be used in my processes to accelerate vulcanization when sulphur, etc. is added. The added sulphur vulcanizes or sulphurizes my modified products further changing their properties.

When making solid vulcanized rubber-like products, I employ temperatures between 120° and 180° C. for vulcanization, and from 5 to 50 parts of sulphur to 100 parts of the isocolloid under treatment. This vulcanization should be effected after modification, and accelerators and antioxidants may be added to the mix in known manner. I may produce liquid vulcanized products as well as rubber-like solids, by regulating the amount of sulphur and the time and temperature of heating. The liquid products are useful as varnish or paint bases.

Two step methods for making vulcanized, modified, heat-bodied fatty oil products are described and claimed in my application Serial No. 236,800 (Patent 2,234,545). As there stated, many of those products are useful as "rubber substitutes." Others are useful for other purposes, for instance, in the manufacture of varnishes, lacquers and other liquid coating compositions, as well as in plastic compositions.

As noted above, the processes may be carried out in various ways, for instance, either in open or closed vessels as desired. In the latter case, the air can be entirely or partially displaced by another gas, such as hydrogen, CO<sub>2</sub>, SO<sub>2</sub>, H<sub>2</sub>S, nitrogen, etc., which influence the results obtained, these gases being used in supplement to the primary modifying agent employed. Again, in both cases such gases may be passed through the material being treated. That is, the modification can be carried out during the passage of a gas. The gas pressure can be that of atmospheric. In many cases, however, a vacuum may be used with advantage. Again, even a higher pressure of several atmospheres is to be recommended in certain cases, it being sometimes advantageous.

That is, I have further found that the results

of the process vary with the nature of the gas present and also with the physical condition (pressure) of this gas. Thus I have found that a certain given starting material which is initially liquid will become slightly viscous only as a result of the modifying treatment, if the latter is effected under atmospheric pressure (open vessel) but more viscous if the gas is rarefied by the employment of a partial vacuum. In other cases the converse applies. When plus pressure was used the results differ again. Air gives a different result from another gas or mixtures of gases such as mentioned ante. The modifying treatment may be carried out either in the total or partial absence of air, by replacing the same with another gas, such as those shown ante.

A pressure treatment followed by a vacuum treatment may be used, and I have found it to be advantageous to use alternately, atmospheric or plus pressure and vacuum treatment. Such alternate treatment increases the uniformity of the distribution of the polar compound in the organic isocolloid. In my processes, the gas may be blown or passed through the liquid mass or simply passed over the surface of the same during the heating. It is advisable in some cases, both when open or closed vessels are employed to have a constant passage of the gas, such as those given ante, during the treatment with the polar compound.

It may be stated with reference to the action of gases, that generally speaking rarefaction of the gases present, by reduction of pressure in the vessel in which the treatment is given, tends to intensify the action of the gases in my processes.

If desired, the polar compound may be produced in situ, that is, within the organic isocolloid under treatment, by interaction within the organic isocolloid, of substances capable of reacting under the conditions of the process to produce the polar compound. The same applies to the gas in the presence of which the organic isocolloid is to be treated and a substance or substances may be added which evolve the desired gas during the processing. It has been found in certain cases that polar compounds and gases which are produced in situ, being in the nascent state, are somewhat more active than those added in the pre-formed state.

As an example of production of the modifying agent in situ, it may be mentioned that salts, such as sodium salts, of various of the sulphonic acids hereinbefore listed may be added to the oil undergoing treatment, as a result of which, during the treatment reaction, the sulphonic acid itself is released, thereby providing for treatment in the presence of a 2-radical type compound, of which the acidic inorganic residue contains sulphur and has the capability of yielding a sulphur-containing acid.

Instead of sodium salts, other alkali metal, alkaline earth metal and heavy metal salts may be used. The alkaline earth metal salts and the heavy metal salts are more advantageous in preparing varnish and paint base materials, than are the salts of alkali metals, because if metal soaps are formed in the oil during the reaction through interchange, the soaps of the alkaline earth metal salts and the heavy metal salts have lower water solubility than do the soaps of the alkali metals. The lower solubility imparts better water resistance properties to paint and varnish films. However, in cases where small proportions of modifying agents are used, even alkali metal salts

may satisfactorily be employed. Examples of the more advantageous metals are barium and lead.

Likewise, the organic isocolloid itself may be formed in situ during the treatment. That is, if it is desired to modify an organic isocolloid which is not a naturally occurring material and which has to be produced before it can be treated, the production of such artificial or manufactured organic isocolloid may be advantageously combined with the treatment with the polar compound. For instance, in making modified heat-bodied fatty oils, the oil may be both heat-bodied and modified in a single step by heat-bodying the fatty oil in the presence of the electrolyte or polar compound. To do this several hours heating at polymerization temperatures is required. Many of my polar compounds are advantageous for this purpose as they accelerate the heat-bodying and polymerization of fatty oils.

In addition to the action of polar compounds and the cooperating action of gases in effecting the colloidal transformations characteristic of my invention, an additional modification of the ultimate physical properties of the treated products can be effected by the addition to the material under treatment, of purely (i. e. metal-free) organic bodies, such as phenols, naphthols, naphthalene, chloroform, acetone, alcohols and their homologues and derivatives. These additions are supplemental to the use of polar compounds. Some of them are solvents and assist in dispersing the polar compound in the organic isocolloid. The use of solvents for this purpose is also shown in my Serial No. 273,159 (Patent 1,985,230) and other prior applications.

I have also found that in my processes the colloidal transformations may be promoted by the use of rays of oscillating energy, such as ultra-violet rays, infra-red rays, X-rays, etc. That is, it is advantageous to irradiate the oil or other organic isocolloid before or during the treatment with the polar compound. Sometimes a subsequent treatment with these rays is also helpful. Further, these rays influence and intensify the action of the gases in my processes.

## EXAMPLES

### Example 1

To 100 parts of rapeseed oil are added 5 parts of naphthalene sulphonic acid and the mixture is heated in a vacuum for two hours to 300-350° C. At the end of this time, the vacuum is broken and the material poured into molds and allowed to cool.

### Example 2

150 parts of linseed oil are heated in vacuum to 280-310° C. for 5 hours with 7.5 parts of 2:5 dichlorbenzene sulphonic acid.

The modified oil product so obtained is a soft solid product suitable for use in making varnishes.

### Example 3

150 parts of linseed oil are heated in an open vessel (at atmospheric pressure) with 7.5 parts of 2:5 dichlorbenzene sulphonic acid to 290-310° C. for 5 hours.

The modified oil product so obtained is a viscous liquid. It is somewhat darker in color than that obtained in Example 2, but it is in some respects more suitable for use in making varnishes.

### Example 4

100 parts of castor oil are heated with 5 parts 2:5 dichlorbenzene sulphonic acid in vacuo at 260° C. for 5 hours.

The modified oil product so obtained is a thick viscous oil, soluble in butyl acetate, in acetone and in benzene.

**Example 5**

1000 parts of castor oil are heated at 270° C. with 50 parts of p-toluene sulphochloride for one hour and then an additional 9000 parts of castor oil are added to the mixture, and this mixture is then held for 2 hours at 270° C., 2 hours at 250° C. 10 and 1 hour at 200° C., during which time a current of nitrogen is bubbled through the so heated mixture.

The modified castor oil product so obtained has a low to medium viscosity and good drying properties. It is a valuable paint and varnish base. 15

**Example 6**

150 parts of linseed oil are heated in an open vessel with 7½ parts of 2:5 dichlorbenzene sulphonate acid to 290-310° C. for 5 hours. The product is a dark viscous liquid, suitable for use 20 as a base for the manufacture of varnishes.

**Example 7**

**COMPARATIVE TESTS**

In this group of tests, alkali refined linseed oil was used and the treating agent employed was 1:4 naphthylamine sulphonic acid (naphthionic acid). 5 to 10 gallon batches of the oil were 30 heated in a varnish kettle in accordance with various different types of cooking methods.

In this group of tests a comparison was always made with a blank control experiment in which the same linseed oil was treated in the same manner, with the one exception that no modifying agent was used. 35

**Test A**

Particularly good results were obtained when employing a CO<sub>2</sub> blanket on the surface of the batch, the batch being agitated during treatment. In this test about 6 hours were required at about 300° C. to reach a viscosity of Z-5 (Gardner scale). This represented a saving of about 30% of the time required to body to the same viscosity, in the absence of the modifying agent. Moreover the oil modified in the presence of the agent was light in color. 40

An ester gum varnish made with the treated oil just referred to was comparable to the blank control experiment in cold and boiling water tests and in cooking time. The modified oil, however, yielded a varnish superior to the varnish made with the blank control oil both in drying and in alkali resistance. 45

The same modified oil was also incorporated in a maleic resin varnish and this varnish bodied in about 20% less time than a similar maleic varnish made with the blank control oil. The varnish made with the modified oil had better drying and alkali resistance than the varnish made with the blank control oil, and the cold and boiling water tests were comparable to the blank control. 50

**Test B**

In accordance with this test 5% of the same reagent (naphthionic acid) was used, the oil being heated for 5 hours at 300° C. at a vacuum of 70 100 mm. of mercury, the batch being agitated. This yielded a light oil of good quality, although with somewhat less body than the oil of Test A. Other properties were similar to the oil produced in accordance with Test A.

**Test C**

In this test agitation was employed, but neither the CO<sub>2</sub> blanket nor the vacuum of Tests A and B were here employed. Various characteristics of the oil were similar, but the color was darker.

**Test D**

Heating procedure similar to that above was employed, but here a CO<sub>2</sub> blanket was employed but no agitation was used. Some charring of the reagent occurred.

**Test E**

Various batches were tried with different percentages of the modifying agent (naphthionic acid), the best results being secured in the range from about .1% up through about .5%. Concentration below about .5% required greater time to secure a given body, whereas concentrations above about .5% had a tendency to char.

**Test F**

Since this particular modifying agent (naphthionic acid) is not readily compatible with the oil, variations in procedure were tried to improve incorporation and dispersing of the reagent in the oil.

In one experiment the desired amount of reagent was mixed thoroughly with water and then added to the oil. In another the reagent was mixed with a small quantity of the oil itself and then this mixture added to the experimental batch. The first method apparently yielded a product of lighter color. 35

**Example 8**

The conditions here employed were similar to those above in Example 7—Test A, but here naphthol sulphonic acid 1:5 (Cleve's acid) was used, the quantity being .5%. As before, the oil was alkali refined linseed oil. The modified oil was not as light as in Example 7, but appreciable improvement, as compared with the blank, in bodying, drying and alkali resistance was indicated. 45

**Example 9**

Here naphthylamine sulphonic acid 2:3:6 (amido R-acid) was used, the heating procedure and percentage being in accordance with that described above in Example 7—Test A. As before, the oil was alkali refined linseed oil. This modifying agent also yields a light oil and improves bodying. 50

**Example 10**

In this experiment sulpho salicylic acid was used with alkali refined linseed oil, and CO<sub>2</sub> bubbled through the oil. The batch was heated for about 2 hours at 300° C., giving a viscosity of Z-4. In cooks using more than .5% of the reagent, the color of the oil was darker than with smaller quantities. 60

**Example 11**

**Test A**

Alkali refined linseed oil was heated for about 2 hours at 300° C. with .5% of beta-naphthol 3:6:8 trisulphonic acid. During the treatment CO<sub>2</sub> was bubbled through the oil. The viscosity was Z-4 and the color fairly dark. 65

**Test B**

Alkali refined linseed oil was heated as in Test A, but with the lead salt of beta-naphthol 3:6:8 trisulphonic acid. The only appreciable differ- 70

ence from Test A was that the bodied oil was lighter in color.

*Test C*

This test is similar to the one just above except for the employment of the barium salt of beta-naphthol 3:6:8 trisulphonic acid. The bodied oil was of lighter color, as in Test B.

Additional experiments were made with a number of other modifying agents, including experiments employing small (fractional) percentages of a modifying agent. Improvement in characteristics of the oils were secured, for instance the drying characteristics and also the bodying. Among other modifying agents tested experimentally the following may be mentioned:

Schaffer salt,  
Anthraquinone-beta-sulphonic acid,  
Oxyquinoline sulphate (yellow),  
Naphthol disulphonic acid 1:3:8 (Andersen's acid),  
Naphthylamine sulphonic acid 2:6:8 (amido G-acid),  
1. naphthylamine 3:6:8 trisulpho acid,  
Naphthalene-beta-sulphonyl chloride,  
2:5 dichlorbenzene-sulphonic acid,  
Naphthol disulphonic acid 1:4:8 (Schoelkopf's acid),  
Naphthol sulphonic acid 1:4 (Neville-Winter acid),  
Naphthol disulphonic acid 2:3:6 (R-salt),  
Laurent's acid.

I claim:

1. In the modification of fatty oils to improve the drying properties thereof, the process which comprises mixing the oil with a minor amount and not more than 10% of a polar compound having within the molecule an organic residue, and an acidic inorganic sulphur-containing residue capable of yielding a sulphur-containing acid at the reaction temperature and in the presence of the reactants present during the treatment, and heating the mixture to a reaction temperature between about 200° and 350° C. for at least thirty minutes.

2. A process in accordance with claim 1 in which the fatty oil is castor oil.

3. A process in accordance with claim 1 in which the fatty oil is linseed oil.
4. In the modification of fatty oils to improve the drying properties thereof, the process which comprises mixing the oil with a minor amount and not more than 10% of a sulphonic acid, and heating the mixture to a reaction temperature between about 200° and 350° C. for at least thirty minutes.
5. A process in accordance with claim 4 in which the fatty oil is castor oil.
6. A process in accordance with claim 4 in which the fatty oil is linseed oil.
7. A process in accordance with claim 4 in which said sulphonic acid is a poly-sulphonic acid.
8. A process in accordance with claim 4 in which said acid is a hydroxy-substituted sulphonate acid.
9. A process in accordance with claim 4 in which said acid is an amino-substituted sulphonate acid.
10. A process in accordance with claim 4 in which said acid is a naphthalene-derivative hydroxy-substituted sulphonate acid.
11. A process in accordance with claim 4 in which said acid is a naphthalene-derivative amino-substituted sulphonate acid.
12. A process in accordance with claim 4 in which said acid is naphthionic acid.
13. A process in accordance with claim 4 in which said acid is beta-naphthol 3:6:8 trisulphonic acid.
14. In the modification of fatty oils to improve the drying properties thereof, the process which comprises mixing the oil with a minor amount and not more than 10% of a salt of a sulphonate acid, and heating the mixture to a reaction temperature between about 200° and 350° C. for at least thirty minutes.
15. In the modification of fatty oils to improve the drying properties thereof, the process which comprises mixing the oil with a minor amount and not more than 10% of a sulphonyl chloride, and heating the mixture to a reaction temperature between about 200° and 350° C. for at least thirty minutes.

LÁSZLÓ AUER.